



US009707791B2

(12) **United States Patent**  
**Fu, Jr. et al.**

(10) **Patent No.:** **US 9,707,791 B2**  
(45) **Date of Patent:** **Jul. 18, 2017**

(54) **PRINTABLE RECORDING MEDIA**

(71) Applicant: **Hewlett-Packard Development Company, L.P.**, Fort Collins, CO (US)

(72) Inventors: **Xulong Fu, Jr.**, San Diego, CA (US); **Xiaoqi Zhou**, San Diego, CA (US); **Francois K. Pirayesh**, San Diego, CA (US); **Lokendra Pal**, San Diego, CA (US)

(73) Assignee: **Hewlett-Packard Development Company, L.P.**, Houston, TX (US)

(\*) Notice: Subject to any disclaimer, the term of this patent is extended or adjusted under 35 U.S.C. 154(b) by 8 days.

(21) Appl. No.: **14/902,523**

(22) PCT Filed: **Jul. 23, 2013**

(86) PCT No.: **PCT/US2013/051640**

§ 371 (c)(1),  
(2) Date: **Dec. 31, 2015**

(87) PCT Pub. No.: **WO2015/012809**

PCT Pub. Date: **Jan. 29, 2015**

(65) **Prior Publication Data**

US 2016/0136985 A1 May 19, 2016

(51) **Int. Cl.**

**B41M 5/50** (2006.01)  
**B41M 5/52** (2006.01)

(Continued)

(52) **U.S. Cl.**

CPC ..... **B41M 5/5254** (2013.01); **B41M 5/502** (2013.01); **B41M 5/506** (2013.01);

(Continued)

(58) **Field of Classification Search**

CPC ..... B41M 5/504; G03C 1/7614  
See application file for complete search history.

(56) **References Cited**

U.S. PATENT DOCUMENTS

5,403,425 A 4/1995 Brown  
6,030,742 A 2/2000 Bourdelais et al.  
(Continued)

FOREIGN PATENT DOCUMENTS

CN 101687422 3/2010  
CN 102333652 1/2012  
(Continued)

OTHER PUBLICATIONS

International Search Report and Written Opinion dated Apr. 29, 2014 for PCT/US2013/051640; Applicant Hewlett-Packard Development Company, L.P.

*Primary Examiner* — Betelhem Shewareged

(74) *Attorney, Agent, or Firm* — HP Inc. Patent Department

(57) **ABSTRACT**

A printable recording media including a supporting base substrate having, on its image side, a pre-coating layer that contains inorganic pigments and polymeric binders, and a top ink-receiving layer that includes inorganic pigments, polymeric binders and non-film forming polymers; and, having a polymer barrier layer on its backside. Also described herein is a method for making the printable recording media, a method for forming printed articles, and the obtained printed articles.

**18 Claims, 2 Drawing Sheets**



|      |                         |                                                                                                                                                                                                                                                                                                                                                                                                                                                                    |             |  |              |                  |         |                        |
|------|-------------------------|--------------------------------------------------------------------------------------------------------------------------------------------------------------------------------------------------------------------------------------------------------------------------------------------------------------------------------------------------------------------------------------------------------------------------------------------------------------------|-------------|--|--------------|------------------|---------|------------------------|
| (51) | <b>Int. Cl.</b>         |                                                                                                                                                                                                                                                                                                                                                                                                                                                                    |             |  |              |                  |         |                        |
|      | <i>G03C 1/76</i>        | (2006.01)                                                                                                                                                                                                                                                                                                                                                                                                                                                          |             |  | 2005/0181185 | A1*              | 8/2005  | Zhou .....             |
|      | <i>B41M 7/00</i>        | (2006.01)                                                                                                                                                                                                                                                                                                                                                                                                                                                          |             |  | 2012/0251717 | A1               | 10/2012 | Zhou et al.            |
|      | <i>G03G 7/00</i>        | (2006.01)                                                                                                                                                                                                                                                                                                                                                                                                                                                          |             |  | 2013/0201251 | A1*              | 8/2013  | Pal .....              |
| (52) | <b>U.S. Cl.</b>         |                                                                                                                                                                                                                                                                                                                                                                                                                                                                    |             |  |              |                  |         |                        |
|      | CPC .....               | <i>B41M 5/5218</i> (2013.01); <i>B41M 5/5227</i> (2013.01); <i>B41M 5/5236</i> (2013.01); <i>B41M 7/0027</i> (2013.01); <i>G03C 1/7614</i> (2013.01); <i>G03G 7/002</i> (2013.01); <i>G03G 7/0013</i> (2013.01); <i>G03G 7/0026</i> (2013.01); <i>G03G 7/0053</i> (2013.01); <i>G03G 7/0086</i> (2013.01); <i>B41M 5/504</i> (2013.01); <i>B41M 2205/34</i> (2013.01); <i>B41M 2205/36</i> (2013.01); <i>B41M 2205/38</i> (2013.01); <i>B41M 2205/40</i> (2013.01) |             |  | 2013/0243977 | A1*              | 9/2013  | Zhou .....             |
|      |                         |                                                                                                                                                                                                                                                                                                                                                                                                                                                                    |             |  |              |                  |         | <i>B41M 5/504</i>      |
|      |                         |                                                                                                                                                                                                                                                                                                                                                                                                                                                                    |             |  |              |                  |         | 428/32.11              |
|      |                         |                                                                                                                                                                                                                                                                                                                                                                                                                                                                    |             |  |              |                  |         | 347/20                 |
|      |                         |                                                                                                                                                                                                                                                                                                                                                                                                                                                                    |             |  |              |                  |         | 428/32.22              |
| (56) | <b>References Cited</b> |                                                                                                                                                                                                                                                                                                                                                                                                                                                                    |             |  |              |                  |         |                        |
|      | U.S. PATENT DOCUMENTS   |                                                                                                                                                                                                                                                                                                                                                                                                                                                                    |             |  |              |                  |         |                        |
|      | 6,030,759 A             | 2/2000                                                                                                                                                                                                                                                                                                                                                                                                                                                             | Gula et al. |  | EP           | 1486346          | 12/2004 |                        |
|      | 7,520,959 B2            | 4/2009                                                                                                                                                                                                                                                                                                                                                                                                                                                             | Kikuchi     |  | JP           | 2005262696       | 9/2005  |                        |
|      |                         |                                                                                                                                                                                                                                                                                                                                                                                                                                                                    |             |  | KR           | 100205164        | 7/1999  |                        |
|      |                         |                                                                                                                                                                                                                                                                                                                                                                                                                                                                    |             |  | KR           | 20050022809      | 3/2005  |                        |
|      |                         |                                                                                                                                                                                                                                                                                                                                                                                                                                                                    |             |  | WO           | 2012057785       | 5/2012  |                        |
|      |                         |                                                                                                                                                                                                                                                                                                                                                                                                                                                                    |             |  | WO           | 2012087334       | 6/2012  |                        |
|      |                         |                                                                                                                                                                                                                                                                                                                                                                                                                                                                    |             |  | WO           | 2013/015767 A1 * | 1/2013  | ..... <i>B41M 5/50</i> |
|      |                         |                                                                                                                                                                                                                                                                                                                                                                                                                                                                    |             |  | WO           | 2013062560       | 5/2013  |                        |

## FOREIGN PATENT DOCUMENTS

|    |                  |         |
|----|------------------|---------|
| EP | 1486346          | 12/2004 |
| JP | 2005262696       | 9/2005  |
| KR | 100205164        | 7/1999  |
| KR | 20050022809      | 3/2005  |
| WO | 2012057785       | 5/2012  |
| WO | 2012087334       | 6/2012  |
| WO | 2013/015767 A1 * | 1/2013  |
| WO | 2013062560       | 5/2013  |

\* cited by examiner



FIG. 1



FIG. 2



FIG. 3

**FIG. 4**

**1**  
**PRINTABLE RECORDING MEDIA**

**BACKGROUND**

Today, images are often captured with a digital camera, transferred electronically to a computer with a printer, or directly to a printer, and then produced by the printer in a hardcopy form. Color inkjet printing and/or laser-jet printing are, among other, often used for printing such high quality photographs. However, in recent years, consumers and businesses have turned to electrophotographic printing systems to produce such digital images on a variety of substrates. Electrophotographic printing systems are using liquid or dry toner electrophotographic ink as ink composition.

It has rapidly become apparent that the image quality of printed images using such printing technology is strongly dependent on the construction of the recording media used. Consequently, improved recording media, often specifically designed, have been developed for use in electrophotographic printing devices. However, while many developments have been made, it has often created challenges to find printable recording media which can be effectively used with electrophotographic printing techniques and which have good image quality as well as good durability. Accordingly, investigations continue into developing such media substrates.

**BRIEF DESCRIPTION OF THE DRAWINGS**

The drawings illustrate various embodiments of the present recording media and are part of the specification.

FIGS. 1 and 2 are cross-sectional views of the printable recording media according to embodiments of the present disclosure.

FIG. 3 is a cross-sectional view of the printed article obtained according to embodiments of the present disclosure.

FIG. 4 is a flowchart illustrating the method for producing a printed article according to some embodiments of the present disclosure.

**DETAILED DESCRIPTION**

Before particular embodiments of the present disclosure are disclosed and described, it is to be understood that the present disclosure is not limited to the particular process and materials disclosed herein. It is also to be understood that the terminology used herein is used for describing particular embodiments only and is not intended to be limiting, as the scope of protection will be defined by the claims and equivalents thereof. In describing and claiming the present article and method, the following terminology will be used: the singular forms "a", "an", and "the" include plural referents unless the context clearly dictates otherwise. Concentrations, amounts, and other numerical data may be presented herein in a range format. It is to be understood that such range format is used merely for convenience and brevity and should be interpreted flexibly to include not only the numerical values explicitly recited as the limits of the range, but also to include all the individual numerical values or sub-ranges encompassed within that range as if each numerical value and sub-range is explicitly recited. For examples, a weight range of about 1 wt % to about 20 wt % should be interpreted to include not only the explicitly recited concentration limits of 1 wt % to 20 wt %, but also to include individual concentrations such as 2 wt %, 3 wt %, 4 wt %, and sub-ranges such as 5 wt % to 15 wt %, 10 wt

% to 20 wt %, etc. All percent are by weight (wt %) unless otherwise indicated. As used herein, "image" refers to marks, signs, symbols, figures, indications, and/or appearances deposited upon a material or substrate with either visible or an invisible ink composition. Examples of an image can include characters, words, numbers, alphanumeric symbols, punctuation, text, lines, underlines, highlights, and the like.

The present disclosure relates to a printable recording media comprising a supporting base substrate having, on its image side, a pre-coating layer that contains inorganic pigments and polymeric binders, and a top ink-receiving layer that includes inorganic pigments, polymeric binders and non-film forming polymers; and, having a polymer barrier layer on its backside. The printable media of the present disclosure is a multi-layer composite structure. The word "composite" refers herein to a material made from at least two constituent materials, or layers, that have different physical and/or chemical properties from one another, and wherein these constituent layers remain separate at a molecular level and distinct within the structure of the composite. The printable recording media encompasses image receiving coatings or top ink-receiving layer. As used herein, the terms "image receiving coating" or "top-coat" are meant to be understood broadly as any coating which can receive an ink or toner; any coating comprising light-sensitive chemicals which, when exposed to a light source, may receive an image; any coating comprising heat sensitive chemicals which, when exposed to heat, may receive an image; or any combination thereof.

In some examples, the printable recording media of the present disclosure is a photographic printing recording media or photo paper recording media, which means herein that the printable recording media is well adapted for photographic printing and that it has the properties and appearances, at least, equal to the properties and appearance of silver halide photo media substrates when image is printed thereon. The printable recording media is thus able to provide advantages such as glossy appearance, surface smoothness and excellent image quality when used to produce photographic printouts. In addition, the printable recording media described herein provides an excellent photobase paper feel. As used herein, the term "photo feel" means that that the printed image feels like a photographic silver halide material when touched.

In some other examples, the printable recording media is an electrophotographic recording media. By electrophotographic recording media, it is meant herein that the media is well adapted for electrophotographic printing processes. The term "electrophotographic printing" is meant to be understood broadly as including any number of methods that use light to produce a change in electrostatic charge distribution to form a photographic image including, but in no way limited to, laser printing. The printable media is thus well-adapted for liquid electrophotographic printing device (i.e. using liquid electrophotographic toner such as, for example, HP Indigo Digital Press 6000 or 6600).

Thus, in yet some other examples, the printable recording media is an electrophotographic photographic recording media. The media can be an electrophotographic photographic recording media for liquid electro-photographic printing (LEP) and can be used in a method of forming photographic printed images. Throughout the various illustrative examples of the present application, the electrophotographic photographic recording media may receive images from printing device such as, for example, an Indigo® WS6000P Digital Printing Press available from Hewlett-

Packard Company (Palo Alto, Calif., USA). Without being linked by any theory, it can be said that, with a six color Indigo® digital printing press WS6000P or 6600P, a user is able to produce photo quality prints comparable to silver halide photo prints. Furthermore, with the use of the printable recording media described herein, there will not need of any additional surface treatment (primer layer) and processing to address inadequate ink or toner adhesion and print uniformity issues to the media, as it is often the case with traditional offset type media.

The printable recording media, described herein, is an image-receiving media that shows excellent print image quality. Said recording media yield not only high gloss appearance but, further, provides a solution to keep the gloss stable under the heat, whether the printers are equipped with single or double heated fuser rollers. In some examples, the printable recording media has a non-imaged gloss which is above about 95 to 100% when tested at 75° angle per Tappi test method of T480, or which is above about 35 to 50% when tested at 60° angle.

The printable recording media, described herein, is consider to lay flat (i.e. having a curl less than 20 mm) across 15° to 30° and 20% to 80% RH condition while achieves good toner adhesion after printing across different user environment. Indeed, photo papers with a curl that is more than 20 mm might result in poor user experiences (issues when trying to display the photo on a table or wall for example). The printable recording media of the present disclosure has an excellent curl control without the need of having a laminate layer on both sides of the media. The printable recording media presents, thus, excellent curl control across different environmental conditions and does not have any curling issues.

Therefore, the recording media described herein has a good surface smoothness, has a high gloss appearance and shows excellent image quality when used to produce photographic printouts. In addition, the recording media has a structure which is receptive and which presents excellent absorption and adherence properties to the ink deposited thereon. The printable recording media enables thus electrophotographic photo printing, such as, for examples, Indigo photo printing, without the need of using any primer composition.

FIG. 1 and FIG. 2 schematically illustrate some embodiments of printable recording media (100). FIG. 3 schematically illustrates some embodiments of a printed article (200). FIG. 4 is a flowchart illustrating the method for producing said printed article (200). As will be appreciated by those skilled in the art, FIG. 1, FIG. 2 and FIG. 3 illustrate the relative positioning of the various layers of the printable media or printed article without necessarily illustrating the relative thicknesses of the various layers. It is to be understood that the thickness of the various layers is exaggerated for illustrative purposes. In some examples, as shown in FIG. 1 or in FIG. 2, the printable media (100) encompasses a base substrate (110); said base substrate (110) can be a paper base substrate. The base substrate has two surfaces: a first surface, which is coated with image-receiving layer which might be referred to as the "image receiving side", "image surface" or "image side" (101), and a second surface, the opposite surface, which might be referred to as the "back surface" or "backside" (102). The image side (101) of the media is the side that includes material layers that will receive, support and protect an image. The backside, or opposing side, (102) does not contains any ink-receiving layer and is not very well adapted to receive the printable image. Without being limited by any theory, it is believed

that coating on the backside (102), when present, might serve to compensate for the presence of the ink-receiving layer on the image side (101) of the base substrate (110). As illustrated in FIG. 1, the printable recording media (100) encompasses a supporting substrate (110), above which is applied a pre-coating layer (120) and a top ink-receiving layer (130). The top ink-receiving layer (130) is applied over said pre-coating layer (120). As illustrated in FIG. 1, the top ink-receiving layer (130) and the pre-coating layer (120), are applied, only, on one side of the supporting substrate (110). On the other side, i.e. backside or opposing side, of the supporting substrate (110), a polymer barrier layer (140) is applied. FIG. 2 illustrates some other embodiments of the printable media (100) wherein the printable media includes pre-coating layers (120) that are applied on both sides of the base substrate (110). The pre-coating layer (120) is thus also present on the backside (102) of the base substrate (110) below the polymer barrier layer (140). FIG. 3 illustrates an example of a printed article (200) according to the present disclosure. The printed article includes a printable media containing a supporting substrate (110) having, on its backside (202), a polymer barrier layer (140) and, on its image side (201), a pre-coating layer (120) and a top ink-receiving layer (130), above which is present a printed image (210). A post-image lamination film (220) is disposed above said printed image (210).

#### Printable Media (100)

##### Supporting Base Substrate (110)

As illustrated in FIG. 1, the printable media (100) contains a supporting base substrate (110) having, on its image side (101), a pre-coating layer (120) and a top ink-receiving layer (130), and having, on its backside (102), a polymer barrier layer (140). The printable media (100) contains a supporting substrate (110) that acts as a bottom substrate layer. The print media substrate (i.e., 'substrate') contains a material that serves as a base upon which the ink-receiving layer is applied. The print media substrate provides integrity for the resultant print medium. The supporting base substrate or raw base substrate (110), on which coating compositions are applied, may take the form of a media sheet or a continuous web suitable for use in a printer. The supporting substrate may be a base paper manufactured from cellulose fibers. The base paper may be produced from chemical pulp, mechanical pulp, thermal mechanical pulp and/or the combination of chemical and mechanical pulp. In some instances, when mechanical pulp is added, the total percentage of mechanical pulp is less than 20% of the total raw base weight. The base paper may also include conventional additives such as retention aid, dry or wet strength agent, internal sizing agents and fillers.

The supporting base substrate (110) can be a cellulose base paper. The raw base substrate (110) can be made of any suitable wood or non-wood pulp. Non-limitative examples of suitable pulps include any kind of chemical pulp, mechanical wood pulp, chemically treated ground pulp, CTMP (chemical thermo mechanical pulp), and/or mixtures thereof. Bleached hardwood chemical pulps may make up the main pulp composition. This pulp has shorter fiber structure than soft wood, which contribute to good formation of the finished paper. In some examples, the raw base substrate (110) contains 100% of chemically treated fiber such as bleached hardwood, softwood fiber, non-wood fiber, synthetic fiber, and combinations. In some other examples, the raw base substrate (110) contains 100% of bleached hardwood and, in yet some other examples, the raw base

substrate (110) contains from about 50 to about 95% of bleached hardwood and from about 5 to about 50 wt % of softwood.

Fillers may be incorporated into the pulp, for example, to substantially control physical properties of the final coated paper. The filler particles fill in the void spaces of the fiber network and result in a denser, smoother, brighter and opaque sheet. Examples of the fillers include, but are not limited to, ground calcium carbonate, precipitated calcium carbonate, titanium dioxide, kaolin clay, silicates, plastic pigment, alumina trihydrate, magnesium oxide and/or mixtures thereof. In some examples, the supporting base substrate contains fillers in an amount ranging from about 0.1 wt % to about 30 wt % of the raw base, and in some other examples, the amount of filler ranges from about 5 wt % to about 15 wt % of the raw base.

When preparing the paper base stock, internal and surface sizing may be used. This process may improve internal bond strength of the substrate fibers, and may control the resistance of the coated substrate to wetting, penetration, and absorption of aqueous liquids. Internal sizing may be accomplished by adding a sizing agent to the raw base in the wet end. Non-limitative examples of suitable sizing agents include rosin-based sizing agent(s), wax-based sizing agent(s), cellulose-reactive sizing agent(s) and other synthetic sizing agent(s), and/or mixtures. In some examples, the internal sizing agents are Alkyl Ketene Dimer (AKD) or alkenylsuccinic anhydride (ASA). It is to be understood that the type and amount of surface sizing agent(s) may substantially improve moisture resistance and may alter the stiffness of the base paper stock. Surface sizing (i.e. apply sizing agent to the paper surface during papermaking process) may be accomplished by film size press, pond size press and other surface techniques. Included in this wet end processing can be additional functional additives such as but not limited to dispersants, biocides, retention aids, defoamers, dyes, and optical brighteners. The raw base substrate (110) can also be surfaced treated with starch or with starch and latex binder with pigments. The surface sizing agent might result in a coat weight of sizing agent in the range of about 0.2 gsm to about 10 gsm.

In some examples, the raw base substrate has a basis weight of about 80 to about 300 gsm, and, in some other examples, has a basis weight of about 150 to about 220 gsm. The stiffness of the raw base can range from about 200 Gurley stiffness units to about 2000 Gurley stiffness units in the paper machine direction, and can range from about 400 Gurley stiffness units and about 1200 Gurley stiffness units in the paper cross machine direction. In some other examples, the base paper stiffness ranges from about 800 Gurley stiffness units to about 1500 Gurley stiffness units in the paper machine direction, and from about 600 Gurley stiffness units to about 1000 Gurley stiffness units in the paper cross machine direction. A method, such as TAPPI T543 om-94, using a Gurley-type stiffness tester, may be used to determine the stiffness of the paper stock. Without being linked by any theory, it is believed that the surface smoothness of the base stock paper is an important factor in the quality of the paper and photographic images printed thereon. A photographic printing base stock with high smoothness and glossiness can be made at effectively low cost, as long as the pigmented sub layer sheets have a minimum smoothness and glossiness level. The surface smoothness can be in the range of from about 0.3 to about 5.0  $\mu\text{m}$ , as measured by a Parker Print Surface (PPS) microprocessor-controlled instrument that performs high

speed, precision measurements of paper surface roughness from Testing Machine Inc. (TMI), New Castle, Del.,

Pre-coating Layer (120)

The printable recording media (100) encompasses a pre-coating layer (120). Said a pre-coating layer (120) is applied above the supporting base substrate (110). Such as illustrated in FIG. 1, the pre-coating layer (120) can be present on one side of the supporting base substrate (110), i.e. on its image side (101); or, such as illustrated in FIG. 2, the pre-coating layer (120) can be present on the backside (102) and on the image side (101) of the recording media (100). In some examples, said pre-coating layer (120) is applied on both sides of the supporting base substrate (110). The pre-coating layer (120) can, thus, be also applied on the backside of the supporting base substrate, below the polymer barrier layer (140).

In some examples, the pre-coating layer (120) is applied over the supporting base substrate (110) with a coat weight of about 2 to about 25 grams/meter<sup>2</sup> (gsm) or with a coat weight ranging from about 10 to about 20 gsm. When applied to both sides of the raw base (110), the coat weight of the pigmented pre-coatings layer (120) can be from about 10 to about 15 gsm for each coating layers. Without being linked by any theory, it is believed that the function of the pre-coating layer (120) is to create a smooth surface to help develop superior gloss. Additionally, the pre-coating layer (120) can promote improved opacity, brightness, and appropriate color hue for the print media.

The pre-coating layer (120) contains at least one inorganic pigment and at least one polymeric binder. In some examples, the inorganic pigment may be prepared in powder or slurry form before being mixed with the binder for coating on the substrate. Examples of inorganic pigments include, but are not limited to, titanium dioxide, hydrated alumina, calcium carbonate, barium sulfate, silica, high brightness alumina silicates, boehmite, pseudo-boehmite, zinc oxide, kaolin clays, and/or their combination. The calcium carbonate may be ground calcium carbonate (GCC) or may be a chemical precipitated calcium carbonate (PCC).

The pre-coating layer (120) may contain from about 40 to about 95 wt % of inorganic pigments by total weight of the layer. Further, with regard to the pigments, the pre-coating layer (120) may include, for example, ground calcium carbonate such as Hydrocarb® 60 available from Omya, Inc.; precipitated calcium carbonate such as Opacarb® A40 or Opacarb® 3000 available from Specialty Minerals Inc. (SMI); clay such as Miragloss® available from Engelhard Corporation; synthetic clay such as hydrous sodium lithium magnesium silicate, such as, for example, Laponite® available from Southern Clay Products Inc., and titanium dioxide (TiO<sub>2</sub>) available from, for example, Sigma-Aldrich Co. The particle size of inorganic pigments can range from about 0.2 to about 1.5 micrometer and, in some other examples, ranges from about 0.5 to about 1.0 micrometer.

The pre-coating layer (120) contains at least one polymeric binder. Without being linked by any theory, it is believed that the function of the binder is to supply an adhesion force between the raw base (110) and the pigment particles, as well as binding pigment particles to each other. The binder may be selected from the group of water-soluble binders and water-dispersible polymers that exhibit high binding power for base paper stock and pigments, either alone or as a combination. Suitable polymeric binders include, but are not limited to, water-soluble polymers such as polyvinyl alcohol, starch derivatives, gelatin, cellulose derivatives, acrylamide polymers, and water-dispersible polymers such as acrylic polymers or copolymers, vinyl

acetate latex, polyesters, vinylidene chloride latex, styrene-butadiene or acrylonitrile-butadiene copolymers. The polymeric binders can be polyvinylalcohol or copolymer of vinylpyrrolidone. The copolymer of vinylpyrrolidone can include various other copolymerized monomers, such as methyl acrylates, methyl methacrylate, ethyl acrylate, hydroxyethyl acrylate, hydroxyethyl methacrylate, ethylene, vinylacetates, vinylimidazole, vinylpyridine, vinylcaprolactams, methyl vinylether, maleic anhydride, vinylamides, vinylchloride, vinylidene chloride, dimethylaminoethyl methacrylate, acrylamide, methacrylamide, acrylonitrile, styrene, acrylic acid, sodium vinylsulfonate, vinylpropionate, and methyl vinylketone, etc. In some examples, the copolymer of vinylpyrrolidone can be a copolymer of vinylpyrrolidone and vinylacetate or vinylcaprolactam or polyvinylalcohol. The polyvinylalcohol or copolymer of vinylpyrrolidone can have a weight average molecular weight ranging from about 10,000 Mw to about 1,000,000 Mw or can have a weight average molecular weight ranging from about 20,000 Mw to about 500,000 Mw. In some examples, the binder is a polyvinylalcohol having a molecular length in the range of 20,000 to 500,000. The inorganic pigment and binder may be used in the following proportions or effective amounts: from 5 to 15 parts by dry weight of binder to 100 parts by dry weight of inorganic pigments. In some other examples, 8 to 10 parts binder are used relative to the 100 parts of pigment.

The pre-coating layer (120) can contain from about 5 to about 40 wt % of water-dispersible binders by total weight of the pre-coating layer and up to 10 wt % of a water-soluble binders. Examples of water-dispersible binders may include, for example, a styrene-butadiene latex such as Gencryl®9780 or PT9619 (from Omnova Solution Inc.); an acrylic polymer sold under the trade name Raycrys® 48083 (available from Specialty Polymers); an aqueous dispersion of an n-butyl acrylate-acrylonitrile-styrene copolymer commercially available under the tradename Acronal®S 504 (available from Baden Aniline and Soda Factory (BASF)); a styrene/n-butyl acrylate copolymer Acronal® S 728 (available from Baden Aniline and Soda Factory (BASF)). In some other examples, the water-dispersible binders have a glass transition temperature (Tg) within the range of about -20° C. to about 35° C. In some other examples, the Tg of the water-dispersible binder is from -10° C. to 0° C. Examples of water-soluble binders may include, for example, a combination of polyvinyl alcohol with methanol sold under the trade name Mowiol®6-98 (available from Kuraray America, Inc.), and 2-hydroxyethyl starch ether sold under the tradename of Penford Gum 280 (available from Penford Products Co.).

In some other examples, the solids content of the coating compositions can range from 60 to 75 percent by weight (wt %) with a viscosity of 1000 to 1500 centipoise (cps) as measured by a low shear Brookfield viscometer at a speed of 100 revolutions per minute (rpm), or 30 cps to 40 cps at a higher shear rate of 4500 rpm using a high shear Hercules viscometer. The pre-coating layer (120) may also include any of the variety of coating additives known to improve the appearance or functionality of media, such as, for examples, mordants, biocides, optical brightener, surfactants, plasticizers, thickeners and cross-linking agents.

#### Top Ink-receiving Layer (130)

The printable media (100) further includes a top ink-receiving layer (130). Said top ink-receiving layer (130) is applied above the supporting base substrate (110), on the image side (101) of the printable media, and can be considered as an image receiving layer. Without being limited

by any theory, it is believed that the top ink-receiving layer (130) is specifically formulated to interact with the ink in order to improve the quality of the printed image. Such top ink-receiving layer (130) can be a liquid electrophotographic printing (LEP) image-receiving layer. By liquid electrophotographic printing (LEP) image-receiving layer, it is meant herein that the layer is adapted to receive image printed using LEP technique, such as printing device using liquid toner manufactured by Hewlett-Packard Company's Indigo press. In some examples, the coat weight of the top ink-receiving layer (130) is ranging from about 5 to about 35 grams/meter<sup>2</sup> (gsm). In some other examples, the coat weight of the top ink-receiving layer (130) is ranging from about 10 to about 20 grams/meter<sup>2</sup> (gsm).

The top ink-receiving layer (130) includes inorganic pigments, polymeric binders and non-film forming polymers. Examples of suitable water-dispersible binders include polybutadiene latex, styrene-butadiene copolymer latex, acrylonitrile-butadiene-styrene terpolymer latex, polychloroprene latex, acrylic latex, polyester emulsions, acrylonitrile-butadiene latex, polyvinyl acetate, polyvinyl acetate copolymers (e.g., vinyl acetate-ethylene latex), and combinations thereof. In some examples, the water-dispersible polymeric binder is a latex binder selected from the group consisting of polybutadiene latex, styrene-butadiene copolymer latex, acrylonitrile-butadiene-styrene terpolymer latex, polychloroprene latex, acrylic latex, polyester emulsions, acrylonitrile-butadiene latex, polyvinyl acetate and polyvinyl acetate copolymers. In some other examples, the water-dispersible polymeric binder is styrene-butadiene copolymer latex. In yet some other examples, the polymeric binder is a carboxylated styrene-butadiene copolymer. In some embodiments, the water-dispersible binders, that are present in the top ink-receiving layer (130), have a glass transition temperature (Tg) within the range of about 0° C. to about 35° C. In some other embodiments, the Tg of the water-dispersible binders, that are present in the top ink-receiving layer (130), is from 10° C. to 30° C. Examples of such water-dispersible polymers include, for example, styrene-butadiene latex such as Gencryl®9780 (available from Omnova Solution Inc.), XU31258.50 (available from Styron Inc.) or Litex®PX 9330 (from Synthomer). The water-dispersible binders can be present, in the top ink-receiving layer (130), in an amount representing from about 10% to about 30% of the total weight of the layer (130).

The top-coat layer (130) may further include a water-soluble binder in addition to the water-dispersible polymers. Suitable water-soluble binders include, but are not limited to polymers such as polyvinyl alcohol, starch derivatives, gelatin, cellulose derivatives, and acrylamide polymers. When present, the amount of water-soluble binder is less than 10 wt % of the total weight of the layer.

The top ink-receiving layer (130) includes inorganic pigments. Suitable inorganic pigments may be provided in a powder or slurry form. Examples of suitable inorganic pigments include, but are not limited to, titanium dioxide, hydrated alumina, calcium carbonate, barium sulfate, silica, clays (such as high brightness kaolin clays), zinc oxide and/or combinations thereof. By way of example only, one suitable inorganic pigment that has desirable properties is calcium carbonate. The calcium carbonate may be one or more of ground calcium carbonate (GCC), precipitated calcium carbonate (PCC), modified GCC and modified PCC. Inorganic pigments are present in the top ink-receiving layer (130) in an amount representing from about 50% to about 90% of the total weight of the layer (130). Examples of inorganic pigments include, but are in no way limited to,

Cartacoat®K (available from Clariant Chemical); Snowtex® ST-O, ST-OL, ST-20L, and ST-C (available from Nissan Chemical); Ludox® CL, AM and TMA (available from Grace-Davison Chemical); Nyacol®AL20, Nyacol®AL20, Nyacol®A1530, Nyacol®Ce02, Nyacol®SN15, Nyacol®DP5370, and NYACOL®Zr50/20 (available from Nyacol Nano Technologies). Examples of inorganic pigments include also GCC, sold under the tradename Hydrocarb®HG or Covercarb®HP (from Omya Inc.) or PCC sold under the tradename Opacarb®A40 (available from Specialty Minerals Inc.).

The polymeric binders that is presents in the top ink-receiving layer (130) can be similar or different from the polymeric binders present in the pre-coating layer (120). In some examples, polymeric binders that are present in the top ink-receiving layer (130) and in the pre-coating layer (120) are water-dispersible binders. In some other examples, the polymeric binders that are present in the top ink-receiving layer (130) and in the pre-coating layer (120) are latex binders selected from the group consisting of polybutadiene latex, styrene-butadiene copolymer latex, acrylonitrile-butadiene-styrene terpolymer latex, polychloroprene latex, acrylic latex, polyester emulsions, acrylonitrile-butadiene latex, polyvinyl acetate and polyvinyl acetate copolymers. In yet some other examples, the polymeric binders that are present in the top ink-receiving layer (130) and in the pre-coating layer (120) are styrene-butadiene copolymer latex.

The top ink-receiving layer (130) includes non-film forming polymers. Non-film forming polymers are water dispersed, polymeric hollow spherical particles filled with water that are non-film forming in ambient conditions and that remain as discrete particles during coating. Such polymers have no substantial coalescence under manufacture and storage conditions. In more details, upon evaporation of the continuous phase (such as solvent and/or water of the dispersed solid-liquid system), the polymers are able to resist deformation and further coalescence. Said polymers can have particulate sizes ranging from about 0.3  $\mu\text{m}$  to about 2  $\mu\text{m}$  and/or a glass transition temperature (Tg) from about 50° C. to about 120° C. In some examples, the glass transition temperature (Tg) for these non-film forming polymers is greater than about 70° C. Such non-film forming polymers can be present in an amount representing from about 5 to about 30 wt % by total weight of the top ink-receiving layer. The ratio between the non-film forming polymer to pigment can be from 1:100 to 1:10.

Non-film forming polymers can be chosen among the group consisting of styrene, acrylic, styrene/acrylics, vinyl/acetate, polyacrylics, methacrylates and combinations thereof. In some examples, the non-film forming polymers are polystyrene latex polymers. In some other examples, the non-film forming polymers are plastic pigment slurry of styrene/butadiene emulsion copolymers. Examples of non-film forming polymers that can be used in accordance with embodiments of the present invention include Ropaque®BC-643, Ropaque®HP-543, or Ropaque®OP-84 (all manufactured by Rohm and Haas Company, USA) and HS-3000NA or HS-3020NA (available from The Dow Chemical Company, USA). Other specific examples of these polymers may include, a styrene acrylic emulsion polymer sold under the trade name Raycat® 29033, a polyacrylic emulsion polymer sold under the trade name Raycat® 78, and an acrylic emulsion polymer sold under the trade name Raycrys® 30S available from Specialty Polymers, Inc. Other examples of such non-film forming polymers include Dow DPPTM 3720 (available from Dow Chemical). Other small

amount of additives such as, for examples, slip aid, deformers, dye, OBA, pH control agent, dispersant and thickener can also be added to the top ink-receiving layer (130).

5 Barrier Layer (140)

The printable media (100) includes a polymer barrier layer (140). Said barrier layer (140) is applied on the supporting base substrate (110), on the backside (102) of the printable media (100). Without being limited by any theory, it is believed that the barrier layer (140) is specifically formulated to provide moisture barrier to the printed article. Furthermore, it is believed that the coat weight of barrier layer (140) on the backside (102) of the media is designed to counter-balance the “pre-stress” generated by the coating layers in the image-receiving side, in other words to be a balance force resulting from the presence of the printed image (210) and of the post-image lamination layer (220). When the polymer barrier layer (140) is applied on the backside (102), the coat weight can be adapted to the weight of the layers present on the image side, so that the final product is curl balanced in all the conditions. In some examples, the higher the thickness of the image side coating and lamination film layers is, the thicker the barrier layer is. The weight ratio between polymer barrier layers to the post printing lamination layer (220) is carefully designed to ensure lay flat of the final printed article/photo. In some example, the ratio between the barrier layer (140) to lamination film layer (220) is from 3:1 to 0.5 to 1. In some examples, the coat weight of the polymer barrier layer (140) is ranging from about 10 to about 60 grams/meter<sup>2</sup> (gsm), in some other examples, is ranging from about 12 to about 45 grams/meter<sup>2</sup> (gsm).

As used herein, the term polymer barrier layer refers to a barrier layer that may contain a polyolefin polymer material, an agro-based polymer material or combinations thereof. The term polyolefin material refers to a polymer produced by olefin homo-polymerization or copolymerization reaction via either high-pressure polymerization or low pressure in the presence of special catalyst like Ziegler and metallocene catalysts, where olefin refers to a hydrocarbon compounds containing a carbon-carbon double bond alkene with general formula  $\text{C}_n\text{H}_{2n}$ . The polymeric barrier coating contains polyolefin resins. Examples of polyolefin resins include, but are not limited to, high density polyethylene (HDPE), low density polyethylene (LDPE), polypropylene (PP), polymethylpentene (PMP), and copolymers of ethylene with hexane, butane, and octane (linear low density polyethylene, LLDPE). The polyolefin resins can also be blends of these polymeric materials, such as HDPE/LDPE, LDPE/LLDPE, PP/LDPE, and PP/LLDPE. In some examples, the polyolefin material that is present in the barrier layer is selected from the group consisting of polyethylene (PE), polypropylene (PP), polymethylpentene, polybutylene polymer, ethylene vinyl acetate polymer and mixtures thereof. In some other examples, the polyolefin material is polyethylene, polypropylene or ethylene vinyl acetate polymer. In yet some other examples, the barrier layer encompasses a low density polyethylene (LDPE), a high density polyethylene (HDPE) or combinations thereof. The barrier layer can encompasses low density polyethylene (LDPE) and high density polyethylene (HDPE) in a ratio that is between 30:70 and 70:30. The polyolefin barrier layer may also encompass polypropylene (PP) and polyethylene terephthalate (PET). The term agro-based material refers to a polymer produced from biomass such as starches, a polymer produced by conventional or

chemical synthesis such as polylactic acid (PLA), or a polymer produced by microbial such as polyhydroxylalcanoates (PHAs).

#### Method for Forming a Printed Article

The printable recording materials are used in printing process in view of forming printed article. In some examples, a method for forming printed articles includes: obtaining a printable recording media (100) comprising a supporting base substrate (110) having, on its image side (101), a pre-coating layer (120) that contains inorganic pigments and polymeric binders, and a top ink-receiving layer (130) that includes inorganic pigments, polymeric binders and non-film forming polymers, and having a polymer barrier layer (140) on its backside; applying an ink composition on the image side of the printable media to form a printed image; and applying a post-image lamination film (220). Such printing method results in printed article (200) with enhanced image quality and enhanced absorption performances. An example of the method for forming printed articles in accordance with the principles described herein, by way of illustration and not limitation, is shown in FIG. 4. FIG. 4 illustrates embodiments of the printing method that encompasses obtaining a printable recording media (100), applying an ink composition onto said media, applying a post-image lamination film (220) and obtaining a printed article (200).

After the images are deposited, established, or printed on the printable media (100), i.e. after an ink layer (210) is formed onto the printable media, a post-image lamination film or laminate layer (220) is disposed. Such post-image lamination film (220) is deposited over the ink, or printed image, that is present on the top image receiving layer (130). In this manner, the laminate layer may provide a final photo finish such as a glossy or matte finish. Further, the laminate layer may provide image durability (such as scratch resistance) and image permanence to the media with what a consumer may consider is a true look and feel of photographic paper. The printed images, resulting from such printing technique, are photo printed image, present high image quality, a good surface smoothness and high gloss appearance.

The post-image lamination film layer (220) can be applied during the printing process (on the press during printing) or can be applied after the printing process using a hot or cold laminator. The post-image lamination film layer (220) can be made of a polyester material or of a polypropylene composition. In some examples, the laminate film (220) is a polyester material. Such polyester material includes, but is not limited to, polyethylene terephthalate (PET), glycol-modified PET, polybutylene terephthalate (PBT), polytrimethylene terephthalate (PTT), polyethylene naphthalate (PEN), polyether terephthalate, polyurethane terephthalate, or a combination or a mixture of two or more thereof. PET may be obtained from Chevron Phillips Chemical Company, The Woodlands, Tex., or from Formosa Plastics Corporation, USA, Livingston, N.J. In some examples, the lamination film is a polypropylene composition. The polypropylene composition contains homo-polymers of polypropylene (PP) and poly(ethylene vinyl acetate) (EVA), for example. Said two components can be coextruded together (i.e., 'PP and EVA'). The PP film polymer and EVA film polymer (either separate or coextruded) may be obtained from film extruder companies and casting companies including, but not limited to, Fabrene, Ontario Canada; Yidu Digital Image company, China. The lamination film is hot laminated to the image layer by a hot laminator. The typical temperature for the hot laminator is about 150° F.

The printable recording media, as described herein, (i.e. comprising a supporting base substrate having, on its image side, a pre-coating layer that contains inorganic pigments and polymeric binders, and a top ink-receiving layer that includes inorganic pigments, polymeric binders and non-film forming polymers; and, having a polymer barrier layer on its backside) contains also a post-image lamination film that is disposed over the top ink-receiving layer after an ink layer is printed. The ink composition may be deposited, established, or printed on the printable media using any suitable printing device. The method for forming printed images can be done by means of digital printing technology. In some examples, the ink may be deposited, established, or otherwise printed on the printable media is a solid toner or a liquid toner. The solid toner or the liquid toner may include toner particles made, e.g., from a polymeric carrier and one or more pigments. The liquid toner may be an organic solvent-based (e.g., hydrocarbon) liquid toner. The solid toner or the liquid toner may be deposited, established, or otherwise printed on the examples of the printable media using, respectively, a suitable dry or liquid press technology, such as a dry toner electrophotographic printing device or a liquid toner electrophotographic printing device. In some other examples, the ink is a liquid electrophotographic ink (liquid toner or liquid ElectroInk) and is applied via electrophotographic printing method. Representative examples of printers used to print on the printable media, include, but are not limited to, Indigo® WS6000P Digital Printing Press or T300 Digital Web Press, both available from Hewlett-Packard Company (Palo Alto, Calif., USA).

Thus, in some embodiments, a method for forming printed articles includes obtaining a printable recording material (100) including a supporting base substrate (110) having, on its image side a pre-coating layer (120) and a top ink-receiving layer (130), and having on its backside a polymer barrier layer (140); providing a liquid electrophotographic ink; applying said ink composition on the image side of the printable media, to form a printed image via electrophotographic printing method; and applying a post-image lamination film (220).

#### The Printed Article

The printed article (200), resulting from the printing process as described above, encompasses, thus, a printable recording material (100) containing a supporting base substrate having, on its image side, a pre-coating layer that contains inorganic pigments and polymeric binders, and a top ink-receiving layer that includes inorganic pigments, polymeric binders and non-film forming polymers, and having a polymer barrier layer on its backside; a printed feature (210) applied on top of said printable recording material, on its image side; and a post-print lamination layer (220) disposed above said printed image. The post-print lamination layer (220), or lamination film, is applied after an ink layer (210) has been printed or otherwise disposed onto the top ink-receiving layer (130) on the image side (101) of the printable media (100) during, for example, the printing process. Without being linked by any theory, it is believed that post-print lamination layer (220), applied to the printed article, provide gloss finish, semi-gloss, luster or matte finish. The lamination film may also provide scratch resistance to the printed article.

As described above, the laminate layer or post-image lamination film (220) can be made of a polyester material or of a polypropylene composition. In some examples, the post-image lamination layer (220) encompasses polyester, polypropylene (PP), PVC, nylon, and other suitable polymer film. In some other examples, the laminate film (220) is a

polyester material. The thickness of the post-print lamination layer (220) can be in the range of from about 10  $\mu\text{m}$  to 60 about  $\mu\text{m}$  (micro); or, in the range of from about 20  $\mu\text{m}$  to 50 about  $\mu\text{m}$ . As mentioned above, the coat-weight ratio of the polymer barrier layer (140) to the laminate layer (220) may be controlled in order to achieve acceptable curl performance across environmental conditions. In some examples, the coat-weight ratio of barrier layer (140), that is applied to the non-image receiving side (101) of the media (100) with respect to the laminate layer (220) that is applied to the image receiving side (202) of the printed article (200), may be between 1:1 and 3:1. In some other examples, the coat weight ratio of the barrier layer (140) to the laminate layer (220) may be 1.5:1. In yet some other examples, the coat-weight ratio of the barrier layer (140) to the laminate layer (220) may be 1.25:1. Thus, in this manner, curling of the printed article (200) may be reduced or eliminated across all environmental conditions including different relative humidities and temperatures.

#### Method for Forming a Printable Recording Material

In some examples, according to the principles described herein, a method of making a printable recording media comprising a supporting base substrate having, on its image side, a pre-coating layer that contains inorganic pigments and polymeric binders, and a top ink-receiving layer that includes inorganic pigments, polymeric binders and non-film forming polymers; and, having a polymer barrier layer on its backside is provided. Such method encompasses providing a supporting base substrate (110); applying a pre-coating layer (120) that contains inorganic pigments and polymeric binders on the raw base substrate on the image side of the supporting base substrate; a top ink-receiving layer (130) that includes inorganic pigments, polymeric binders and non-film forming polymers, over said pre-coating layer; drying and calendering said pre-coating layer and top ink-receiving layer and extruding a polymer barrier layer (140) on the backside of the supporting base substrate. In some examples, the pre-coating layer (120) is applied to the supporting base substrate on the image receiving side and on the backside of the printable media.

The pre-coating layer (120) and the top ink-receiving layer (130) are thus coated to the image side (102) and the pre-coating layer (120) is coated to the backside (102) of the base substrates (110). Such pre-coating layer (120) and top ink-receiving layer (130) can be applied using an on-machine or off-machine coater. Examples of suitable coating techniques include slotted die application, roller application, curtain coater, blade application, rod application, air knife application, gravure application, airbrush application, and others known in the arts. In some examples, the pre-coating layer(s) (120) are coated using an offline coater, or applied during raw base paper making process. The top ink-receiving layer (130) can be applied using in line or offline coater such as blade coater, roll coater, slot, or curtain coater. The solids content of the top ink-receiving layer (130) can range from about 20 wt % to about 68 wt % depending on coating method used, with a viscosity of about 100 cps to about 2000 cps as measured by low shear Brookfield viscometer at a speed of about 100 rpm. The coat layer can then be dried by convection, conduction, infrared radiation, atmospheric exposure, or other known method.

After coating the base stock with the top ink-receiving layer (130), a calendering process can be used to achieve desired gloss or surface smoothness. The calendering device can be a separate super calendering machine, an on-line soft nip calendering unit, an off-line soft nip calendering machine, or the like. Super-calendering is calendering in a

calender unit in which nips are formed between a smooth-surface press roll, such as a metal roll, and a roll covered with a resilient cover, such as a polymer roll. The resilient-surface roll adapts itself to the contours of the surface of paper and presses the opposite side of paper evenly against the smooth-surface press roll. Any of a number of calendering devices and methods can be used. The calendering device can be a separate super-calendering machine, an on-line calendering unit, an off-line soft nip calendering machine, or the like. Some calendering systems do not require the paper to be as completely dried as other forms of calendering. In some examples, the calendering is carried out at a temperature ranging from about 50 to about 220° C. (metal roll surface temperature) and, in some other examples, from about 100 to about 170° C. The nip pressure can be any value between about 50 to about 300 Kg/cm<sup>2</sup>. The roughness, on the image side (101) of the printable recording media, after calendar process can be less than 3 micro, and less than 6 micro for the backside (102) on the image side of the printable recording media, per Park Print Surface method (PPS method).

The polymer barrier layer (140) can be applied according to various extrusion operations like extrusion coating, lamination, hot melt extrusion or modification of cast extrusion or coating operation. In some examples, the barrier layer is applied on the backside of the base substrate with the use of a heat melted extrusion coating processing. The polymer barrier layer is extrusion coated on the backside of the supporting base substrate with a coat weight ranging from about 12 to about 50 grams/meter<sup>2</sup> (gsm), or with a coat weight ranging from about 20 to about 30 gsm. In some examples, the polymer barrier layer (140) is formed by a co-extrusion process. The barrier layer can also be made by hot melt extrusion technique. As used herein, the terms extrude and hot melt extrusion refer to process wherein the material is heated to a temperature at, or above, its melting point and deposited on a moving substrate at a uniform thickness. In some examples, in the extrusion process, the material is heated to a considerably higher temperature than its melting point. The extrusion process may be practiced within a wide range of extrusion temperatures, for example, from about 310° C. to about 350° C. in case of polyethylene, and speeds, for example, from about 60 m/min to about 460 m/min. In such extrusion processes, the component of the barrier layer is first subjected to heat and pressure inside the barrel of an extruder. The molten polymer is then forced through the narrow slot of an extrusion-coating die by an extruder screw. At the exit of the slot die, a molten curtain emerges. In some examples, this molten curtain is drawn down from the die into a nip between two counter-rotating rolls, a chill roll and pressure roll. In some other examples, while coming into contact with a faster moving substrate in the nip formed between the chill roll and the pressure roller, a hot film is drawn out to the desired thickness, forming a layer with a specific thickness onto the substrate

#### EXAMPLES

##### Ingredients:

TABLE 1

| Ingredient name   | Nature of the ingredients | supplier  |
|-------------------|---------------------------|-----------|
| Hydrocarb ®60 MEZ | GCC pigment               | Omya Inc. |

TABLE 1-continued

| Ingredient name  | Nature of the ingredients                                               | supplier             |
|------------------|-------------------------------------------------------------------------|----------------------|
| Opacarb ®3000    | PCC pigment                                                             | SMI                  |
| Litex ®PX 9330   | Polymer Latex (Tg of 22° C.) (carboxylated styrene/butadiene copolymer) | Synthomer            |
| Gencryl PT ®9619 | Styrene butadiene Polymer Latex (Tg of -6° C.)                          | Omnova Solution Inc. |
| Dow DPP ®3720    | polystyrene latex                                                       | Dow                  |
| Mowiol ®6-98     | PVOH                                                                    | KSE                  |
| Ca-stearate      | lubricant                                                               | Greven               |
| Alcogum ®L265    | Thickener                                                               | Alco Chemicals       |
| Sterocoll ®BL    | Thickener                                                               | BASF                 |

## Example 1

## Preparation of the Media

Pre-coat layer and top ink-receiving layer formulations 1 and 2 are prepared by mixing the ingredients as illustrated in table 2. Media A and B are printable media according to the present disclosure. Media A and B both contain a raw base substrate (110), a pre-coating layer (120) applied on both sides of said raw base, a top ink-receiving layer (130) applied over the pre-coating layer (120) on the image side of the media and a polymer barrier layer (140) applied over the pre-coating layer (120) on the backside of the recording media. The raw base is made with base paper stock prepared with cellulose fibers. Such base paper stock contains about 60% of hardwood, about 20% of softwood and about 10% of calcium carbonate fillers. The raw base is surface sized with oxidized starch. The pickup rate for the starch is 1 gsm each side.

Pre-coating layers (120) are applied on the image side raw base with a coat weight of about 12 gsm. Top-coating layer (130) is applied over said pre-coating layers (120) on the image side of the printable media. The pre-coating and top-coat formulations are illustrated in the table 2 below. The pre-coating and top coat are applied with a lab blade coater at a coat weight of about 12 gsm. The media is then calendered with a lab soft calender at 1000 psi and 100 deg. C. The final smoothness of the recording media is about 1 micro per PPS method. The barrier layer (140) is applied to the backside of said raw base substrate by extrusion coating or lamination process. The formula of the different coatings, used for making the media A and B, are illustrated in the table 2 below.

TABLE 2

|                                              | Formulation 1<br>MEDIA A | Formulation 2<br>MEDIA B |
|----------------------------------------------|--------------------------|--------------------------|
| Base paper (110) (in wt %)                   |                          |                          |
| hardwood fiber                               | 60.0%                    | 60.0%                    |
| softwood fiber                               | 20.0%                    | 20.0%                    |
| calcium carbonate                            | 10.0%                    | 10.0%                    |
| Pre-coating layer (120) (in part per weight) |                          |                          |
| Hydrocarb ®60 MEZ                            | 65                       | 65                       |
| Opacarb ®3000                                | 35                       | 35                       |
| Litex ® PX 9330-Tg of 22° C.                 | 9                        | —                        |
| Gencryl PT ®9619 Tg of -6° C.                | —                        | 9                        |
| Mowiol ®6-98                                 | 1                        | 1                        |
| Defoamer                                     | 0.042                    | 0.042                    |

TABLE 2-continued

|    |                                                                          | Formulation 1<br>MEDIA A | Formulation 2<br>MEDIA B |
|----|--------------------------------------------------------------------------|--------------------------|--------------------------|
| 5  | Alcogum L261                                                             | 0.13                     | 0.13                     |
|    | Sterocoll BL                                                             | 0.047                    | 0.047                    |
|    | NaOH                                                                     | 0.06                     | 0.06                     |
|    | Top ink-receiving layer (130) (in part per weight)                       |                          |                          |
| 10 | Opacarb ®3000                                                            | 100                      | 100                      |
|    | Litex ® PX 9330 (Tg of 22° C.)                                           | 9                        | —                        |
|    | Gencryl ®PT ®961 (Tg of -6° C.)                                          | —                        | 9                        |
|    | Dow DPP ®3720                                                            | 3                        | 3                        |
|    | Mowiol ®6-98                                                             | 1                        | 1                        |
|    | Defoamer                                                                 | 0.044                    | 0.044                    |
|    | Ca-stearate                                                              | 0                        | 0                        |
| 15 | Alcogum ®L265                                                            | 0.146                    | 0.146                    |
|    | Sterocoll BL                                                             | 0.017                    | 0.017                    |
|    | NaOH                                                                     | 0.06                     | 0.06                     |
|    | Barrier layer (140) (CTW = 25 gsm with 50:50 ratio of HD/LD PE) (in gsm) |                          |                          |
| 20 | HDPE                                                                     | 12.5 gsm                 | 12.5 gsm                 |
|    | LDPE                                                                     | 12.5 gsm                 | 12.5 gsm                 |

The structures and compositions of media A, B, and C are illustrated in the table 3 below. Media A and B are printable recording media according to the present disclosure; Media C is a comparative examples that does not have a barrier layer. The table summarizes the coat weight of the different layers, when present, in gram/square meter (gsm).

TABLE 3

|    | media A                       | media B | Comparative media C |
|----|-------------------------------|---------|---------------------|
| 30 | Base Paper                    | 150 gsm | 150 gsm             |
|    | Image side                    |         |                     |
| 35 | Pre-coating layer (120)       | 12 gsm  | 12 gsm              |
|    | Top ink-receiving layer (130) | 12 gsm  | 12 gsm              |
|    | Backside                      |         |                     |
| 40 | Pre-coating layer (120)       | 3 gsm   | 3 gsm               |
|    | Barrier layer (140)           | 25 gsm  | 25 gsm              |

The media A, B and C are printed on HP Indigo press WS6000 to check ink adhesion. A post-image lamination film is applied to both printed media with a hot lamination process (100° C.). Two types of lamination films are used: BOPP and PET as illustrated in table 4.

TABLE 4

|                                  | media A  | media B |
|----------------------------------|----------|---------|
| Post-image Lamination film (220) |          |         |
| 50                               | JNP BOPP | 29 µm   |
|                                  | Yidu PET | —       |
| 55                               |          | 32 µm   |

## Example 2

## Printable Recording Media Performances

The media are evaluated for their curling effect and for their adhesion performances. The curling effect is evaluated by preparing, at least three sheets of the different samples A and C (either in 4"×6" size sheet). The samples are then acclimate on wire rack in various environment conditions chammers such as 23° C. at 50% Relative Humidity (RH);

32° C. at 20% RH; 15° C. at 80% RH; 15° C. at 20% RH; 30° C. at 80% RH for 24 hours. The samples are then measured: the four curling edges are measured using ruler. Such measures are reported in mm (“+” defines curls forming towards the image layer side and “-” defines curls forming away from the image layer side). The average of the curl is then calculated for each condition. The absence of curling or a small curling effect is obtained when measures are close to zero. An absence of curling effect is desired. The results are shown in table 5 below. It demonstrates that the comparative Media C has very poor curl performances while media A exhibits an excellent curl performance across all environmental conditions tested.

TABLE 5

| Curling at different temperature/humidity condition (in mm) |               |               |               |               |               |
|-------------------------------------------------------------|---------------|---------------|---------------|---------------|---------------|
|                                                             | 23° C. at 50% | 15° C. at 20% | 32° C. at 20% | 15° C. at 80% | 30° C. at 80% |
| media A                                                     | +2            | -2            | -5            | +17           | +18           |
| media C                                                     | +36           | +37           | +47           | +100          | +100          |

The ink/toner adhesion is measured by using a 3M tape. The tape is placed on the imaged sample. After the tape is pulled off the image, the OD loss is measured. The acceptable toner adhesion for photo application is less than 15% OD loss after 1 hour printing. One hour after printing, both sample A and B are tested for toner adhesion at different time interval (0 min, 15 min and 1 hour) for the different colors. The KOD is the black optical density, the COD is the optical density for the cyan color, the MOD is the optical density for the magenta color and the YOD is the optical density for the yellow color. Table 6 below shows the OD retained compared to the control (OD measured before toner adhesion test) after the tape is pulled off from the image. The results demonstrate that media A has good adhesion performance while sample B showed poorer toner adhesion.

TABLE 6

|                         | KOD   | COD   | MOD   | YOD   |
|-------------------------|-------|-------|-------|-------|
| MEDIA A (formulation 1) |       |       |       |       |
| control                 | 1.417 | 0.638 | 1.577 | 1.106 |
| 0 min                   | 1.016 | 0.428 | 1.114 | 0.802 |
| 15 min                  | 1.371 | 0.607 | 1.117 | 1.073 |
| 60 min                  | 1.446 | 0.645 | 1.286 | 1.108 |
| MEDIA B (formulation 2) |       |       |       |       |
| control                 | 1.407 | 0.631 | 1.569 | 1.086 |
| 0 min                   | 0.52  | 0.395 | 0.737 | 0.519 |
| 15 min                  | 0.631 | 0.395 | 0.535 | 0.548 |
| 60 min                  | 0.75  | 0.505 | 0.555 | 0.772 |

The invention claimed is:

1. A printable recording media comprising a supporting base substrate having:

a. on its image side,

- a pre-coating layer that contains inorganic pigments and polymeric binders,
- and a top ink-receiving layer that includes inorganic pigments, polymeric binders and non-film forming polymers, wherein a weight ratio of non-film forming polymer to inorganic pigments in the top ink-receiving layer is from 1:100 to 1:10;

b. and having a polymer barrier layer on its backside.

2. The printable recording media according to claim 1 wherein the pre-coating layer is also applied on the backside of the supporting base substrate, below the polymer barrier layer.

3. The printable recording media according to claim 1 wherein the polymeric binders, present in the top ink-receiving layer and in the pre-coating layer, are latex binders selected from the group consisting of polybutadiene latex, styrene-butadiene copolymer latex, acrylonitrile-butadiene styrene terpolymer latex, polychloroprene latex, acrylic latex, polyester emulsions, acrylonitrile-butadiene latex, polyvinyl acetate and polyvinyl acetate copolymers.

4. The printable recording media according to claim 1 wherein the polymeric binders, present in the top ink-receiving layer and in the pre-coating layer, are styrene-butadiene copolymer latex.

5. The printable recording media according to claim 1 wherein the polymeric binders, in the top ink-receiving layer, are water-dispersible binders and are present in an amount representing from about 10 wt % to about 30 wt % of the total weight of the layer.

6. The printable recording media according to claim 1 wherein the polymeric binders, in the top ink-receiving layer, are water-dispersible polymeric binders and have a glass transition temperature (Tg) within the range of about 0° C. to about 35° C.

7. The printable recording media according to claim 1 wherein the polymeric binders, in the pre-coating layer, are polyvinylalcohol or copolymer of vinylpyrrolidone.

8. The printable recording media according to claim 1 wherein the non-film forming polymers, present in the top ink-receiving layer, have a glass transition temperature (Tg) which is above about 70° C.

9. The printable recording media according to claim 1 wherein the non-film forming polymers, present in the top ink-receiving layer, are chosen among the group consisting of styrene, acrylic, styrene/acrylics, vinyl/acetate, polyacrylics, methacrylates and combinations thereof.

10. The printable recording media according to claim 1 wherein a post-image lamination film is disposed over the top ink-receiving layer after an ink layer is printed.

11. The printable recording media according to claim 10 wherein the post-image lamination film is made of a polyester material or of a polypropylene composition.

12. A method for forming printed articles comprising:  
a. obtaining a printable recording media comprising a supporting base substrate having, on its image side, a pre-coating layer that contains inorganic pigments and polymeric binders, and a top ink-receiving layer that includes inorganic pigments, polymeric binders and non-film forming polymers, wherein a weight ratio of non-film forming polymer to inorganic pigments in the top ink-receiving layer is from 1:100 to 1:10; and, having a polymer barrier layer on its backside;

b. applying an ink composition on the image side of the printable media, to form a printed image;

c. and applying a post-image lamination film.

13. The method for forming printed articles according to claim 12 wherein the ink composition is a liquid electro-photographic ink.

14. A printed article obtained according to the method of claim 12 comprising:

a. a printable recording media with a supporting base substrate having, on its image side, a pre-coating layer that contains inorganic pigments and polymeric binders, and a top ink-receiving layer that includes inorganic pigments, polymeric binders and non-film form-

**19**

- ing polymers, wherein a weight ratio of non-film forming polymer to inorganic pigments in the top ink-receiving layer is from 1:100 to 1:10; and, having a polymer barrier layer on its backside;
- b. a printed feature applied on top of said printable recording material, on its image side;
- c. and a post-image lamination film disposed above said printed feature.
- 15.** A method for making a printable recording material comprising:
- providing a supporting base substrate;
  - applying a pre-coating layer that contains inorganic pigments and polymeric binders on the raw base substrate on the image side of the supporting base substrate;
  - applying a top ink-receiving layer, that includes inorganic pigments, polymeric binders and non-film forming polymers, over said pre-coating layer, wherein a

**20**

- weight ratio of non-film forming polymer to inorganic pigments in the top ink-receiving layer is from 1:100 to 1:10;
- d. drying and calendaring said pre-coating layer and top ink-receiving layer;
- e. and extruding a polymer barrier layer on the backside of the supporting base substrate.
- 16.** The printable recording media according to claim **1**, wherein the polymer barrier layer comprises a blend of high density polyethylene and low density polyethylene.
- 17.** The printable recording media according to claim **16**, wherein a weight ratio of high density polyethylene to low density polyethylene in the barrier layer is from 30:70 to 70:30.
- 18.** The printable recording media according to claim **1**, wherein the polymer barrier layer has a coat weight from about 10 gsm to about 60 gsm.

\* \* \* \* \*